

# UNITED STATES PATENT OFFICE.

EDWARD GOODRICH ACHESON, OF STAMFORD TOWNSHIP, ONTARIO,  
CANADA, ASSIGNOR TO WILLIAM ACHESON SMITH, OF NIAGARA  
FALLS, NEW YORK.

## REFRACTORY ARTICLE AND METHOD OF MAKING THE SAME.

No. 836,853.

Specification of Letters Patent.

Patented Nov. 20, 1906.

Application filed September 23, 1905. Serial No. 279,855.

*To all whom it may concern:*

Be it known that I, EDWARD GOODRICH ACHESON, a citizen of the United States, residing in Stamford township, Ontario, Canada, have invented certain new and useful Improvements in Refractory Articles and Method of Making the Same, of which the following is a specification.

The present invention relates to the production of crucibles or other refractory coherent articles or bodies of a compound of silicon, carbon, and oxygen.

The invention comprises both the method of producing such articles and the product thereof.

In manufacturing fire-bricks by molding a moistened mass of finely-divided siloxicon, which is a compound of silicon, carbon, and oxygen, and firing to develop the self-bonding property, as disclosed in my Patent No. 722,793, of March 17, 1903, I have noticed that when the bricks are heated in an oxidizing atmosphere the surface is harder and tougher than the interior. I therefore concluded that the action of oxygen increases the self-bonding property.

The present invention is based on this observation that the self-bonding property of silicon, carbon, and oxygen is increased by the action of oxygen.

In carrying out my present invention I mold or otherwise shape the compound of silicon, carbon, and oxygen into a body and fire it under oxidizing conditions throughout the body. For this purpose the finely-divided compound is preferably mixed with a small amount of an oxidizing agent. It is desirable that the oxidizing agent thus added should not liberate its oxygen at a low temperature. Agents which have been found suitable for the purpose are metallic oxids, such as those of manganese, iron, or chromium. The presence of free carbon in the mixture or the addition of carbon thereto is not detrimental to the self-bonding property. In practice the articles may be produced by employing ninety-two parts, by weight, of the compound of silicon, carbon, and oxygen—for example, siloxicon—one part of manganese dioxid, seven parts of carbon, and a sufficient amount of a liquid—such as water, petroleum, or glycerin—or a viscous one, such as water and dextrine, to bring the mass

into a plastic state. The constituents are preferably finely divided and intimately 55 mixed. The mixture is then shaped in any usual way and fired, preferably at a red heat.

In order to subject the article to a high and uniform temperature, it is preferably embedded in carbon and fired in an electric furnace. 60

While it is to be understood that the precise nature of the effect produced by the oxidizing agent and of the free carbon, if present, is not accurately known and that the 65 scope of this invention is independent of theory, it has been found that the above materials furnish a mixture which is well adapted for the purposes intended. Crucibles have thus been produced which on account 70 of their high heat conductivity, chemical inertness, and durability are especially suitable for the use of steel and brass founders.

While the described method is that preferably employed, articles of sufficient strength 75 for many uses may be made by simply molding a mixture of the finely-divided compound of silicon, carbon, and oxygen with a temporary binder and firing the mixture under oxidizing conditions throughout the body—as, 80 for instance, in an atmosphere of compressed oxygen.

I claim—

1. The process of producing refractory coherent articles, which consists in shaping a 85 mass of a compound of silicon, carbon and oxygen and firing the shaped body under oxidizing conditions throughout the body.

2. The process of producing refractory coherent articles, which consists in mixing a 90 finely-divided compound of silicon, carbon and oxygen with an oxidizing agent, molding the mixture and firing the molded body.

3. The process of producing refractory coherent articles, which consists in mixing a 95 finely-divided compound of silicon, carbon and oxygen with a metallic oxid, molding the mixture and firing the molded body.

4. The process of producing refractory coherent articles, which consists in mixing a 100 finely-divided compound of silicon, carbon and oxygen with an oxidizing agent and carbon, molding the mixture and firing the molded body.

5. As a new manufacture, an article consisting of a molded and fired body of particles 105

- of a compound of silicon, carbon and oxygen, the component particles having been subjected to oxidizing conditions during the firing.
5. As a new manufacture, an article consisting of a shaped and fired mixture of a compound of silicon, carbon and oxygen and an oxidizing agent.
7. As a new manufacture, an article consisting of a shaped and fired mixture of a compound of silicon, carbon and oxygen, an oxidizing agent and carbon.
8. As a new manufacture, an article con-
- sisting of a molded and fired mixture of a compound of silicon, carbon and oxygen and a metallic oxid. 15
9. As a new manufacture, an article consisting of a molded and fired mixture of a compound of silicon, carbon and oxygen, a metallic oxid and carbon. 20

In testimony whereof I affix my signature in presence of two witnesses.

EDWARD GOODRICH ACHESON.

Witnesses:

EUGENE A. BYRNES,  
F. L. FREEMAN.